

Patented July 8, 1924.

1,500,954

# UNITED STATES PATENT OFFICE.

WALTHER MATHESIUS AND HANS MATHESIUS, OF CHARLOTTENBURG, GERMANY.

## MANUFACTURE OF LEAD ALLOYS.

No Drawing.

Application filed October 21, 1922. Serial No. 596,128.

To all whom it may concern:

Be it known that we, WALTHER MATHESIUS and HANS MATHESIUS, German subjects, residing in Charlottenburg, Germany, 5 have invented a certain new and useful Manufacture of Lead Alloys, of which the following is a specification.

For some years there have been used in substitution for the previously usual tin 10 bearing-alloys, alloys of hardened lead. These alloys consist of lead which has been hardened by introduction of alkaline earth metal or alkali metal.

The scientific investigation of these alloys 15 has shown that in their production are formed chemical compounds of lead with the aforesaid metals of the type  $PbCa_3$ , which are soluble in the lead and which separate when cooled either as primary crystals or in 20 eutectic form. These compounds of lead are essentially harder than the pure metal and therefore when the alloy is used as a bearing-metal the compounds become after short use of the bearing, the true bearing 25 surface on which the shaft rests.

The resistance to wear of such a bearing surface depends on the hardness and resistance of these metal compounds.

It has been attempted to introduce into 30 such bearing metals, copper as such or in the form of a copper-tin alloy, in order to bring about the formation of still harder alloys and thus to enhance the resistance to wear, of the bearing surface.

Generally speaking, the result is only satisfactory so long as small proportions of copper are added to the metal bath; as soon as the addition is increased, faults in the 35 castings begin to appear since the separation of the copper crystals from the solution in the lead begins at a relatively high temperature, before the alkaline earth metal or alkali metal compounds of lead begin to crystallize. The whole mass of bearing 40 metal is then so liquid that even in the comparatively short time during which the metal remains in the pot, casting ladle or the like, there is opportunity for copper or copper-tin particles to rise to the surface of the bath and there to form particles of semi-solid alloy.

This defect can be avoided according to the present invention by introducing the copper into the bath in the form of a compound of copper and calcium ( $CuCa_4$ ) or a

corresponding copper compound of another alkaline earth metal or alkali metal.

It is then possible to produce alloys of the aforesaid kind with a content of 4 to 6% or more of copper which, even on long standing in fused condition do not show segregation. The explanation of this exceptional behaviour of the copper is revealed by metallographic investigation of a photograph, from which it can easily be seen that in such 65 alloys the copper is contained in the form of the new alloy constituent, namely in small salmon-coloured crystals which occur in quite preponderating proportion on those 70 surfaces of the polished specimen that are formed of lead-calcium crystals or lead-calcium-strontium crystals. If the alloy contains barium also, the eutectic lead-barium alloy surrounding the lead-calcium crystals is nearly completely free from copper-calcium 75 crystals.

For a simple method of preparation of the alloy above referred to, containing 4 to 6% of copper, and having the desired properties above referred to, the following is given:

63 parts of lead are melted in a pot and 37 parts of calcium are added thereto, and the mixture well stirred, in order to produce the alloy having substantially the composition represented by the formula  $PbCa_3$ . The pot containing the alloy is kept at somewhat above the melting point, and about 15 to 22 parts of calcium cupride, the alloy having the composition represented by the formula  $CuCa_4$ , are added thereto, while the mass is being stirred or mixed in the melting pot. The entire mass of alloy in the melting pot can then be allowed to cool or can be poured into suitable molds in order to form bearings 95 for shafts or the like. It will be seen that in this example, the alloy  $CuCa_4$  is added as such to the alloy  $PbCa_3$ , the two being mixed together in a molten state.

While the above particular example relates especially to the use of calcium cupride,  $CuCa_4$ , it will be understood that other compounds of this type can be used, as represented hereinafter by the general formula  $CuM_4$ , in which M represents an atom of an 100 alkaline earth metal or the equivalent of an alkali metal.

From the foregoing property of the polished specimen it follows that during the cooling the copper-calcium crystals separate 110

from the total alloy almost simultaneously with the lead-calcium crystals and therefore owing to the large quantity of the latter are prevented from segregating by rising to the 5 surface. There is thus obtained a completely new kind of bearing metal which contains small and very much harder copper-calcium crystals in very large number within the lead-calcium crystals.

10 These copper-calcium crystals form in the metal the true bearing surface which in consequence of the great hardness of the said crystals has a very much greater resistance to wear than has an alloy which 15 contains as hardening constituents only compounds of lead with alkali metals or alkaline earth metals.

It is noteworthy that, as can be ascertained by metallographic investigation, copper 20 per-calcium crystals are not formed when copper is added as such to a previously formed alkaline earth metal bearing-metal, even when this addition is in the form of molten copper or of a highly heated solution 25 of copper in lead.

On the other hand, another method of causing a bearing metal of the kind in question to take up copper as a permanent admixture consists in dissolving copper at a 30 sufficiently high temperature in lead and in introducing into this molten mass the necessary alkali metal or alkaline earth metal by electrolytic separation of the latter.

During the long period of action at high 35 temperature of the alkali metal or alkaline earth metal separated in statu nascendi on the lead bath, the copper particles dissolve and appear to combine chemically with the calcium or other electrolytically separated 40 alkali or alkaline earth metal. From the fact that the alkali or alkaline earth metal compounds of copper formed in this way are not decomposed again by the large mass of the lead present in excess, it must be deduced that the chemical affinity of the copper 45 for the electrolytically separated metal is somewhat greater than that of the lead.

This excess of energy, however, is not sufficiently great to render possible the production of the corresponding copper-metal compounds when copper is added to the hardened lead alloy, i. e., an alloy of lead with an alkali or an alkaline earth metal.

On the other hand, a practical, very complete and convenient method of introducing the copper into the lead bearing-metal consists in making the latter by electrolysis and adding to the electrolyte a copper salt suitable for the particular condition of the electrolysis in suitable proportion, for instance cupric chloride or cuprous chloride.

In the appended claims the term "alkali-forming metal" is used to embrace alkali metals and alkaline earth metals. The ex-

pression "metallic lead material" is used to embrace both pure metallic lead as well as alloys of this containing alkali metal or alkaline earth metal.

We claim:

1. An alloy containing lead as its major constituent together with smaller amounts of an alkali-forming metal and copper, such copper being added in the form of a compound thereof with an alkali-forming metal. 70

2. An alloy containing lead as its major constituent together with smaller amounts of an alkali-forming metal and copper, the amount of copper in said alloy being not below 4%, and the amount of the alkali-forming metal being more than four atoms 75 to each atom of copper, the copper being in the form of a compound with the alkali-forming metal. 80

3. A process of making an alloy containing lead as its major constituent and smaller 85 amounts of an alkali-forming metal and copper, by adding a molten compound of copper with an alkali-forming metal to a molten metallic lead material, and stirring.

4. A process of making an alloy containing lead as its major constituent and smaller amounts of an alkali-forming metal and copper, by adding a molten compound of copper with an alkali-forming metal to a molten metallic lead material, and stirring. 90

5. A lead bearing-metal hardened by the presence of a small percentage of an alkali-forming metal and containing incorporated in it, copper in the form of a compound of copper with an alkali-forming metal of the type  $CuM_4$ . 100

6. The method of making an alloy for bearings, wherein copper is added in the form of a compound of copper of the type  $CuM_4$  to a previously made fused, lead-containing bearing-metal and uniformly distributed therein by a thorough stirring. 105

7. A method as defined in claim 6, in which the copper compound is added in a molten condition. 110

8. In the manufacture of lead alloys, the step of introducing into the molten mass, an alloy containing about one atom of copper to four atoms of alkali-forming metal.

9. A bearing metal composed essentially of lead, an alkali-forming metal and copper, the copper being united with some of the alkali-forming metal as a crystalline compound of the typical formula  $CuM_4$ , such crystalline material being homogeneously distributed throughout the remaining constituents of the alloy, the amount of copper in said alloy being much less than the amount of lead. 115

In testimony whereof we have signed our 120 names to this specification.

WALTHER MATHESIUS. [L. s.]  
HANS MATHESIUS. [L. s.]